# EUROPEAN PATENT SPECIFICATION

(11) **EP 1 800 771 B1**
(45) Date of publication and mention of the grant of the patent: **20.04.2011**
(21) Application number: 06126676.3
(22) Date of filing: 20.12.2006
(51) Int. Cl.: B22C 1/14

(54) **A moulding material and a method for casting, and an additive for the moulding material**
Stoffzusammensetzung von Sandform und Giessereiverfahren und Sandformadditiv
Sable de fonderie et méthode de coulée ainsi qu'un additif carboné pour sable de fonderie

(30) Priority: 22.12.2005 SE 0502882
(43) Date of publication of application: 27.06.2007
(73) Proprietor: Swerea SWECAST AB, 550 02 Jönköping (SE)
(72) Inventor: Nayström, Peter, 560 27, TENHULT (SE)
(74) Representative: Bokinge, Ole

(56) References cited:
- EP-A- 0 476 966
- EP-A- 0 814 147
- FR-A1- 2 377 244
- US-A1- 2 830 913
- US-B2- 6 860 319
- LANDIS C R: "Analytical Pyrolysis for Detection of Benzen Detection of Benzen Potential in Sand-System Coals" NEW TECHNOLOGY, AMERICAN FOUNDRYMEN'S SOCIETY, DES PLAINES, IL, US, no. 110, 1996, pages 865-871, XP002075764 ISSN: 0099-4251
- EMILY C. RUBENSTEIN, GRADUATE THESIS: "casting environmental governance: the evolution of regulatory relationships in the wisconsin foundry industry" 2002, MASSACHUSETTS INSTITUTE OF TECHNOLOGY (MIT) , XP002425587 * paragraph [CHAPTER.II.PART.F.THE.CO.EDUCTAION.PROCES S] * * paragraph [BRIDGING.PAGES.32.AND.33] *
- "National emission standards for Hazardous Air Pollutants (NESHAP) for Iron and Steel Foundries - Background Information for Proposed Standards" October 2002 (2002-10), OFFICE OF AIR QUALITY PLANNING AND STANDARDS (OAQPS) OF THE UNITED STATES ENVIRONMENTAL PROTECTION AGENCY (EPA) , SPRINGFIELD USA , XP002425588 * paragraph [6.5.2.CONTINUOUS.VOC.MONITORING.SYSTEMS] * * tables 5.4.Summary.of.ORGANIC.HAP.EMISSION,SOURCE ,TEST * * paragraph [APPENDIX.C] *
- LAFAY VICTOR, HILL AND GRIFFITH COMPANY: "green sand - The process of the future" DUCTILE IRON NEWS, vol. 3, 2005, pages 1-12, XP002424780 Ohio, USA
- LAFAY VICTOR, NELTER S., HILL AND GRIFFITH COMPANY: "Understanding Emissions in green sand molding" AFS TRANSACTIONS, 2002, pages 1-41, XP002424781
- LAFAY VICTOR ET AL.: "Evaluating Emission characteristics of seacoal and seacoal supplements using advanced analytical techniques" AFS TRANSACTIONS, vol. 46, 2000, pages 713-718, XP002424782 Ohio, USA

## Description

### Field of the Invention

The present invention relates to a moulding material and a method for casting iron, the moulding material containing sand and a carbonaceous material, which comprises pit coal. The invention further concerns an additive for a moulding material, the additive containing a carbonaceous material which comprises pit coal.

### Background

In the casting of iron in green sand moulds, it is known to form a moulding material that contains about 80-90% by weight of sand, about 5-11% by weight of binder (usually bentonite), about 3-4% by weight of water and about 2-6% by weight of carbonaceous material.

In commercially used moulding materials, the carbonaceous material consists mainly of powdered coal, or alternatively a coal dust replacement. A problem associated with this kind of carbonaceous material is that it contains a certain amount, usually about 30% by weight, of volatile compounds (such as VOC - volatile organic compounds), which are set free as the moulding material is heated, and which cause emissions from the foundry plant. However, these volatile organic compounds have a beneficial effect on the casting performance by reducing the adherence of, for example, the moulding material to the cast object, thus reducing the amount of moulding sand that has to be removed from the cast object in subsequent production stages.

In Dempsey, LaFay, Neltner, Taulbee: Understanding Properties of Carbonaceous Additives and Their Potential to Emit Benzene, AFS Transactions, 97-107, pp. 109-117, a casting method is shown in which anthracite, metallurgical coke and lignite are added to a mixture of carbonaceous material, the main component of which is pit coal.

In LaFay, Neltner, Taulbee, Wellbruck, Ashburn: Applying Emission Characteristics of Seacoal and Seacoal Supplements for the Foundry Industry, AFTS Transactions, 99-23, pp. 7-10, casting methods are shown in which a carbonaceous material that contains respectively about one half of pit coal and one half of natural asphalt (Gilsonite) and one half of pit coal and one half of anthracite.

In LaFay, Neltner, Taulbee, Wellbrock, Ashburn: Evaluating Benzene Emissions During Casting of Aluminum and Iron, AFS Transactions, 99-01, pp. 745-750, a casting method is shown in which 2% pit coal is added to the moulding material.

In LaFay, Neltner, Taulbee, Wellbrock: Evaluating Emission Characteristics of Seacoal and Seacoal Supplements Using Advanced Analytical Techniques, AFS Transactions, 00-46, pp. 713-718, a casting method is shown in which 2% carbonaceous material is added to the moulding material and in which the percentages of weight of the carbonaceous material are about 67% anthracite and 22% pit coal.

In LaFay, Neltner: Green Sand Without Seacoal, AFS Transactions, 04-111, pp. 671-681, casting methods are shown in which cellulose, anthracite and lignite are analyzed as substitutes for pit coal, and in which it is found that wholly replacing the pit coal will result in reduced casting performance (adherence of sand).

In Moore, Brown: Coal in Greensand Systems - A new look at a very old practice, Foundry Trade Journal, June 2005, an admixture of 3-5% coke to the moulding material is shown.

US 5,688,313 discloses an activated carbon and/or activated graphite foundry sand additive, and method of casting molten metal against a foundry sand containing the additive composition.

Accordingly, there is a need for an improved moulding material and an improved casting method, which combine low emissions of volatile organic compounds with reduced adherence of sand to the cast article.

### Summary of the Invention

An object of the present invention is to provide a moulding material, a method for casting and an additive for such a moulding material, which partly or entirely eliminate the problems associated with prior art. A particular object is to provide a moulding material, a casting process and an additive, which reduce the emissions of volatile organic compounds, in combination with a low adherence of sand to the cast article.

The invention is defined in the appended independent claims. Embodiments are outlined in the dependent claims and in the following description.

Thus, a moulding material for casting iron is provided, which moulding material contains sand and a carbonaceous material, the carbonaceous material constituting 0.5-10% by weight of the moulding material and containing pit coal. The carbonaceous material contains, relatively to each of the components of the carbonaceous material, mainly coke in proportion by weight.

A moulding material of this kind can be made acceptable in terms of both emissions and the adherence of moulding material to the cast object.

According to embodiments, 40% by weight or more, preferably 50% by weight or more, of the carbonaceous material, can be coke. The lower limit for the amount of coke is not critical for the performance of the moulding sand in terms of adherence, but can be chosen based on the permissible amount of emissions.

According to further embodiments, 60% by weight or more, preferably 70% by weight or more, of the carbonaceous material can be coke.

According to further embodiments, 99% by weight or less, preferably 95% by weight or less, 90% by weight or less, 80% by weight or less, 75% by weight or less or 70% by weight or less, of the carbonaceous material can be coke.

According to further embodiments, the remaining part of the carbonaceous material can be pit coal, or pit coal and coal dust replacement.

According to embodiments, 30% by weight or less, preferably 20% by weight or less, 15% by weight or less, 10% by weight or less, of the carbonaceous material can be pit coal, or pit coal and coal dust replacement.

According to further embodiments, the moulding material can contain 25% by weight or less, preferably 6% by weight or less, 4% by weight or less or 2.5% by weight or less, of carbonaceous material.

According to further embodiments, the moulding material can contain 0.5% by weight or more, 1% by weight or more, 1.5% by weight or more, 2% by weight or more, 2.5% by weight or more, 3% by weight or more, 3.5% by weight or more, 4% by weight or more or 4.5% by weight or more, of carbonaceous material.

According to further embodiments, the moulding material can contain a binder, for example about 4-15% by weight, preferably 5-11% by weight, of binder. The binder can be bentonite.

According to further embodiments, the moulding material can contain graphite, preferably in an amount of up to about 0.5-2% by weight of the moulding material. By adding graphite the moulding material is made more fluid and thus becomes easier to handle.

According to further embodiments, the remaining part of the moulding material, in addition to the components referred to above, can be sand, which part preferably constitutes 80-95% by weight, preferably 80-90% by weight of the moulding material.

According to a second aspect, use of a moulding material as described above for casting iron objects is provided.

According to a third aspect, a process is provided for casting iron in a moulding material containing sand and a carbonaceous material, which constitutes 0.5% by weight of the moulding material and comprises pit coal. The process comprises mixing coke into the moulding material, so that the main component by weight of the carbonaceous material, in proportion to each of the components of the carbonaceous material, is coke.

According to a fourth aspect, an additive for a moulding material intended for casting iron is provided. The additive contains a carbonaceous material comprising pit coal and is distinguished in that the carbonaceous material, relatively to each of the components of the carbonaceous material, mainly contains coke in proportion by weight.

According to one embodiment, the remaining part of the carbonaceous material of the additive is pit coal, or pit coal and coal dust replacement.

According to one embodiment, the additive contains a binder.

According to one embodiment, the binder comprises bentonite.

According to one embodiment, the additive contains graphite.

The advantages obtained by means of the additive described above will be apparent, for example, from the above description of the moulding material according to the invention. Moreover, the conceivable amounts contained in the additive will be apparent from said description and the description below.

### Description of Embodiments

Tests were made consisting in the casting of brake discs of grey cast iron with a weight of 6.2 kg. A basic mixture for a moulding material, consisting of synthetic moulding sand, mixed from virgin materials, was prepared, wherein quartz-felspar was mixed with 5% by weight of soda-treated calcium bentonite and water, and then stored for one month. The amount of water was chosen so as to provide a suitable consistency of the moulding sand, and the amount of added water was about 2.3-3.1% by weight. The basic mixture was mixed with different additives. The final amount of sand (percentage by dry weight) can be calculated from the tables below, since it constitutes the remaining part not stated in the tables. All weight parts in the tables relate to the dry weight composition of the mixtures.

Additions to the basic mixture of moulding sand were made according to the following:

In a first sample, "Sample 1", a moulding material made up of a basic mixture and 4% by weight of coke was prepared. The carbonaceous material in this moulding material thus consisted of 100% by weight coke.

In a second sample, "Sample 2", a moulding material made up of a basic mixture, 3% by weight coke and 1% by weight graphite. The carbonaceous material in this moulding material thus consisted of 75% by weight coke and 25% by weight graphite.

In a third sample, "Sample 3", a moulding material made up of a basic mixture and 4% by weight of powdered coal. The carbonaceous material in this moulding material thus consisted of 100% by weight of powdered coal.

In a fourth sample, "Sample 4", use was made of a commercially used circulating, i.e. recycled, moulding material, with a measured carbon content of about 4.5% by weight. The carbonaceous material added in this moulding material was made up of powdered coal and coal dust replacement. Furthermore, this moulding material contains, due to the circulation, a small amount of coke, which is formed when the moulding material is heated during casting and the powdered coal and coal dust replacement are converted into coke. In addition, this moulding material contains carbonaceous rests from polymere-containing binders used during the manufacture of mould cores.

In a fifth sample, "Sample 5", a moulding sand made up of a basic mixture and 4% by weight coke and 1.5% by weight of powdered coal was prepared. The carbonaceous material in this moulding material thus consisted of 73% by weight coke and 27% by weight powdered coal.

In a sixth sample, "Sample 6", the moulding material of Sample 2 was used, wherein 0.5% by weight powdered coal was added. The carbonaceous material in this moulding material thus consisted of 67% by weight coke, 22% by weight graphite and 11% by weight powdered coal.

In a seventh sample, "Sample 7", the moulding material of Sample 2 was used, wherein a basic mixture was added to obtain a total amount of coke representing 1.5% by weight and a total amount of graphite representing 0.5% by weight. Furthermore, 0.5% by weight of powdered coal was added. The carbonaceous material in this moulding material thus consisted of 60% by weight coke, 20% by weight graphite and 20% by weight powdered coal.

In an eighth sample, "Sample 8", a moulding material according to the EU project GO-APIC (Proj. No. G1RD-CT-2000-00235) was used. The carbonaceous material in this moulding material was made up of a graphite-zeolite blend, and thus contained no coke.

Upon casting, the cast article was left to cool for 40 minutes in the mould, following which one form part was removed and placed on its end on the other form part for 20 minutes, to allow volatile organic compounds set free by the form parts to be collected by the ventilating hood and measured in the ventilating duct.

After a total time of one hour, the cast article was separated from the moulds and vibrated on a separating device for one minute, and then left to cool completely.

When the cast articles had reached room temperature, they were vibrated for another minute on the separating device and then blasted. Weighing of the cast articles was carried out after the first minute on the separating device.

In samples 1-4, the volatile organic compounds were measured by means of a ventilating hood provided with FID instruments, which measure the content of volatile organic compounds in the ventilating duct. Furthermore, the amount of sand was measured after the first separation.

In sample 8, only the amount of sand was measured following the first separation. Table 1 shows the results of the measurements for Samples 1-4.

**Table 1: Results for Samples 1-4**

| Sample | | 1 | 2 | 3 | 4 |
|---|---|---|---|---|---|
| Bentonite | [% by weight] | 5.1 | 5.1 | 5.1 | 6.5 |
| Coke | [% by weight] | 4 | 3 | 0 | -* |
| Pit coal/ Coal dust replacement | [% by weight] | 0 | 0 | 4 | -* |
| Graphite | [% by weight] | 0 | 1 | 0 | -* |
| Carbon content | [% by weight] | 3.2 | 2.9 | 3.0 | 4.5 |
| VOC max | [ppm] | 0.05 | 0.01 | 24 | 19 |
| Sand amount | [% by weight] | 8.5 | 6.2 | 1.7 | 2.2 |

| | | | | | |
|---|---|---|---|---|---|
| * No content data available, since the sample was a reference sample with recycled moulding material. | | | | | |

Samples 1-4 and 8 are comparative examples and do not form part of the claimed invention.

Table 1 shows that a moulding material with no admixture of pit coal results in an unacceptably large amount of adhering moulding material. Thus, Samples 1 and 2 are unacceptable from the point of view of productivity, since an excessive amount of adhering sand is obtained.

Table 1 further shows that a moulding material in which pit coal constitutes a small proportion of the carbonaceous material results in low emissions of volatile organic compounds. Thus, Samples 3 and 4 are unacceptable from the point of view of emissions.

Table 2 illustrates the results of the measurements for Samples 5-8.

**Table 2: Results for Samples 5-8**

| Sample | | 5 | 6 | 7 | 8 |
|---|---|---|---|---|---|
| Bentonite | [% by weight] | 5.1 | 5.1 | 5.1 | 6.8 |
| Coke | [% by weight] | 4 | 3 | 1.5 | 0 |
| Hard coal/ Coal dust replacement | [% by weight] | 1.5 | 0.5 | 0.5 | 0 |
| Graphite | [% by weight] | 0 | 1 | 0.5 | < 2.0 |
| Carbon content | [% by weight] | 4,1 | 3.2 | 1.9 | < 1.0 |
| Sand amount | [% by weight] | 1.3 | 3.0 | 6.6 | 6.0 |

Table 2 shows that a moulding material in which the main component of the carbonaceous material is coke, with the admixture of pit coal, results in an acceptable amount of adhering moulding material.

Because the emissions of volatile organic compounds are directly proportional to the amount of powdered coal/coal dust replacement, it is found that Samples 5-7 should be acceptable also from the point of view of emissions.

Thus, the conclusion is that a moulding material which contains sand and carbonaceous material, and in which the carbonaceous material contains pit coal and/or coal dust replacement, the main component of the carbonaceous material being coke, can be made acceptable both in terms of emissions and in terms of adherence.

The extensive adherence of moulding material in Sample 7 is likely due to the fact that the total amount of carbonaceous material was too small, approximately 1.9% by weight. A likely remedy to this problem would be to add more coke, thereby increasing the carbon content. Another measure available would be to add zeolites, as shown, for example, in EP-1 469 960 A1.

## Claims

1. A moulding material for casting iron, which moulding material contains sand and a carbonaceous material, the carbonaceous material constituting 0.5-10% by weight of the moulding material and containing pit coal, **characterised in that** the carbonaceous material, relatively to each of the components of the carbonaceous material, contains mainly coke in proportion by weight.

2. A moulding material according to claim 1, wherein 40% by weight or more, preferably 50% by weight or more, of the carbonaceous material is coke.

3. A moulding material according to claim 2, wherein 60% by weight or more, preferably 70% by weight or more, of the carbonaceous material is coke.

4. A moulding material according to any one of the preceding claims, wherein less than 99% by weight, preferably 95% by weight or less, 90% by weight or less, 80% by weight or less, 75% by weight or less or 70% by weight or less, of the carbonaceous material is coke.

5. A moulding material according to any one of claims 1, 3 and 4, wherein the remaining part of the carbonaceous material is pit coal, or pit coal and coal dust replacement.

6. A moulding material according to claim 5, wherein less than 30% by weight, preferably 20% by weight or less, 15% by weight or less, 10% by weight or less, of the carbonaceous material is pit coal, or pit coal and coal dust replacement.

7. A moulding material according to any one of the receding claims, wherein the moulding material contains 10% by weight or less, preferably 6% by weight or less, 4% by weight or less or 2.5% by weight or less, of carbonaceous material.

8. A moulding material according to any one of claims 1-6, wherein the moulding material contains 0.5% by weight or more, 1% by weight or more, 1.5% by weight or more, 2% by weight or more, 2.5% by weight or more, 3% by weight or more, 3.5% by weight or more, 4% by weight or more or 4.5% by weight or more, of carbonaceous material.

9. A moulding material according to any one of the preceding claims, wherein the moulding material contains a binder.

10. A moulding material according to claim 9, wherein the moulding material contains about 4-15% by weight, preferably 5-11% by weight, of binder.

11. A moulding material according to claim 9 or 10, wherein the binder comprises bentonite.

12. A moulding material according to any one of the preceding claims, wherein the moulding material contains graphite, preferably in an amount of up to about 0.5-2% by weight of the moulding material.

13. A moulding material according to any one of the preceding claims, wherein the remaining part of the moulding material is sand, which part preferably constitutes 80-95% by weight, preferably 80-90% by weight, of the moulding material.

14. Use of a moulding material according to any one of the preceding claims.

15. A method for casting iron in a moulding material containing sand and a carbonaceous material, which constitutes 0.5-10% by weight of the moulding material and comprises pit coal, **characterised in that** the method comprises mixing coke into the moulding material, so that the main component of the carbonaceous material in proportion by weight, relatively to each of the components of the carbonaceous material, is coke.

16. An additive for a moulding material intended for casting iron, which additive contains a carbonaceous material comprising pit coal, **characterised in that** the carbonaceous material, relatively to each of the components of the carbonaceous material, contains mainly coke in proportion by weight.

17. An additive according to claim 16, wherein the remaining part of the carbonaceous material is pit coal, or pit coal and coal dust replacement.

18. An additive according to claim 16 or 17, wherein the additive contains a binder.

19. An additive according to claim 18, wherein the binder comprises bentonite.

20. An additive according to claims 16-19, wherein the additive contains graphite.

## Patentansprüche

1. Eine Formmasse für Eisenguss, die Sand und ein kohlenstoffhaltiges Material enthält, wobei das kohlenstoffhaltige Material 0,5-10 Gew.-% der Formmasse ausmacht und Steinkohle enthält, **dadurch gekennzeichnet, dass** das kohlenstoffhaltige Material, verhältnismäßig zu jedem der Bestandteile des kohlenstoffhaltigen Materials, bezogen auf das Gewicht hauptsächlich Koks enthält.

2. Eine Formmasse nach Anspruch 1, worin 40 Gew.-% oder mehr, vorzugsweise 50 Gew.-% oder mehr des kohlenstoffhaltigen Materials Koks ist.

3. Eine Formmasse nach Anspruch 2, worin 60 Gew.-% oder mehr, vorzugsweise 70 Gew.-% oder mehr des kohlenstoffhaltigen Materials Koks ist.

4. Eine Formmasse nach irgendeinem der vorhergehenden Ansprüche, worin weniger als 99 Gew.-%, vorzugsweise 95 Gew.-% oder weniger, 90 Gew.-% oder weniger, 80 Gew.-% oder weniger, 75 Gew.-% oder weniger, oder 70 Gew.-% oder weniger des kohlenstoffhaltigen Materials Koks ist.

5. Eine Formmasse nach irgendeinem der Ansprüche 1, 3 und 4, worin der übrige Teil des kohlenstoffhaltigen Materials Steinkohle ist, oder Steinkohle und Kohlenstaub-Ersatz.

6. Eine Formmasse nach Anspruch 5, worin weniger als 30 Gew.-%, vorzugsweise 20 Gew.-% oder weniger, 15 Gew.-% oder weniger, 10 Gew.-% oder weniger des kohlenstoffhaltigen Materials Steinkohle ist, oder Steinkohle und Kohlenstaub-Ersatz.

7. Eine Formmasse nach irgendeinem der vorhergehenden Ansprüche, worin die Formmasse 10 Gew.-% oder weniger, vorzugsweise 6 Gew.-% oder weniger, 4 Gew.-% oder weniger, oder 2,5 Gew.-% oder weniger des kohlenstoffhaltigen Materials enthält.

8. Eine Formmasse nach irgendeinem der Ansprüche 1-6, worin die Formmasse 0,5 Gew.-% oder mehr, 1 Gew.-% oder mehr, 1,5 Gew.-% oder mehr, 2 Gew.-% oder mehr, 2,5 Gew.-% oder mehr, 3 Gew.-% oder mehr, 3,5 Gew.-% oder mehr, 4 Gew.-% oder mehr, oder 4,5 Gew.-% oder mehr des kohlenstoffhaltigen Materials enthält.

9. Eine Formmasse nach irgendeinem der vorhergehenden Ansprüche, worin die Formmasse ein Bindemittel enthält.

10. Eine Formmasse nach Anspruch 9, worin die Formmasse ungefähr 4-15 Gew.-%, vorzugsweise 5-11 Gew.-% Bindemittel enthält.

11. Eine Formmasse nach Anspruch 9 oder 10, worin das Bindemittel Betonit enthält.

12. Eine Formmasse nach irgendeinem der vorhergehenden Ansprüche, worin die Formmasse Graphit enthält, vorzugsweise in einer Menge von bis zu ungefähr 0,5-2 Gew.-% der Formmasse.

13. Eine Formmasse nach irgendeinem der vorhergehenden Ansprüche, worin der übrige Teil der Formmasse Sand ist, wobei dieser Teil vorzugsweise 80-95 Gew.-%, vorzugsweise 80-90 Gew.-% der Formmasse ausmacht.

14. Verwendung einer Formmasse nach irgendeinem der vorhergehenden Ansprüche.

15. Ein Verfahren für Eisenguss in einer Formmasse, welche Sand und ein kohlenstoffhaltiges Material enthält, das 0,5-10 Gew.-% der Formmasse ausmacht und Steinkohle enthält, **dadurch gekennzeichnet, dass** das Verfahren Mischen von Koks in die Formmasse umfasst, so dass die Hauptkomponente des kohlenstoffhaltigen Materials, verhältnismäßig zu jedem der Bestandteile des kohlenstoffhaltigen Materials, bezogen auf das Gewicht hauptsächlich Koks ist.

16. Ein Zusatz für eine Formmasse, die für Eisenguss bestimmt ist, wobei der Zusatz ein kohlenstoffhaltiges Material enthält, das Steinkohlekohle enthält, **dadurch gekennzeichnet, dass** das kohlenstoffhaltige Material, verhältnismäßig zu jedem der Bestandteile des kohlenstoffhaltigen Materials, bezogen auf das Gewicht hauptsächlich Koks enthält.

17. Ein Zusatz nach Anspruch 16, worin der übrige Teil des kohlenstoffhaltigen Materials Steinkohle ist, oder Steinkohle und Kohlenstaub-Ersatz.

18. Ein Zusatz nach Anspruch 16 oder 17, worin der Zusatz ein Bindemittel enthält.

19. Ein Zusatz nach Anspruch 18, worin das Bindemittel Bentonit enthält.

20. Ein Zusatz nach Ansprüchen 16-19, worin der Zusatz Graphit enthält.

## Revendications

1. Sable de fonderie pour coulée de fonte, le sable de fonderie contenant du sable et une substance carbonée, la substance carbonée constituant 0,5 % à 10 % en poids du sable de fonderie et contenant du charbon minéral, **caractérisé en ce que** la substance carbonée, relativement à chacune des composantes de la substance carbonée contient principalement du coke dans une proportion en poids.

2. Sable de fonderie selon la revendication 1, dans lequel 40 % en poids ou plus, de préférence 50 % en poids ou plus, de la substance carbonée est du coke.

3. Sable de fonderie selon la revendication 2, dans lequel 60 % en poids ou plus, de préférence 70 % en poids ou plus, de la substance carbonée est du coke.

4. Sable de fonderie selon l'une quelconque des revendications précédentes, dans lequel moins de 99 % en poids, de préférence 95 % en poids ou moins, 90 % en poids ou moins, 80 % en poids ou moins, 75 % en poids ou moins ou 70 % en poids ou moins, de la substance carbonée est du coke.

5. Sable de fonderie selon l'une quelconque des revendications 1, 3 et 4, dans lequel la partie restante de la substance carbonée est du charbon minéral ou du charbon minéral et un substitut de poussière de charbon.

6. Sable de fonderie selon la revendication 5, dans lequel moins de 30 % en poids, de préférence 20 % en poids ou moins, 15 % en poids ou moins, 10 % en poids ou moins, de la substance carbonée est du charbon minéral, ou du charbon minéral et un substitut de poussière de charbon.

7. Sable de fonderie selon l'une quelconque des revendications précédentes, dans lequel le sable de fonderie contient 10 % en poids ou moins, de préférence 6 % en poids ou moins, 4 % en poids ou moins ou 2,5 % en poids ou moins, de substance carbonée.

8. Sable de fonderie selon l'une quelconque des revendications 1 à 6, dans lequel le sable de fonderie contient 0,5 % en poids ou plus, 1 % en poids ou plus, 1,5 % en poids ou plus, 2 % en poids ou plus, 2,5 % en poids ou plus, 3 % en poids ou plus, 3,5 % en poids ou plus, 4 % en poids ou plus ou 4,5 % en poids ou plus, d'additif carboné.

9. Sable de fonderie selon l'une quelconque des revendications précédentes, dans lequel le sable de fonderie contient un agent liant.

10. Sable de fonderie selon la revendication 9, dans lequel le sable de fonderie contient environ 4 % à 15 % en poids, de préférence 5 % à 11 % en poids, d'agent liant.

11. Sable de fonderie selon la revendication 9 ou 10, dans lequel l'agent liant comprend de la bentonite.

12. Sable de fonderie selon l'une quelconque des revendications précédentes, dans lequel le sable de fonderie contient du graphite, de préférence dans une quantité pouvant atteindre environ 0,5 % à 2 % en poids du sable de fonderie.

13. Sable de fonderie selon l'une quelconque des revendications précédentes, dans lequel la partie restante du sable de fonderie est du sable, cette partie constituant de préférence 80 % à 95 % en poids, de préférence 80 % à 90 % en poids, du sable de fonderie.

14. Utilisation d'un sable de fonderie selon l'une quelconque des revendications précédentes.

15. Procédé de coulée de fonte dans un sable de fonderie contenant du sable et une substance carbonée qui constitue 0,5 % à 10 % en poids du sable de fonderie et comprend du charbon minéral, **caractérisé en ce que** le procédé comprend le fait de mélanger du coke dans le sable de fonderie, de telle sorte que le composant principal de la substance carbonée dans une proportion en poids, relativement à chacune des composantes de la substance carbonée, est du coke.

16. Additif pour un sable de fonderie destiné à couler de la fonte, l'additif contenant une substance carbonée comprenant du charbon minéral, **caractérisé en ce que** la substance carbonée, relativement à chacune des composantes de l'additif carboné contient principalement du coke dans une proportion en poids.

17. Additif selon la revendication 16, dans lequel la partie restante de la substance carbonée est du charbon minéral, ou du charbon minéral et un substitut de poussière de charbon.

18. Additif selon la revendication 16 ou 17, dans lequel l'additif contient un agent liant.

19. Additif selon la revendication 18, dans lequel l'agent liant comprend de la bentonite.

20. Additif selon les revendications 16 à 19, dans lequel l'additif contient du graphite.
